

1

2,894,865

**METHOD OF IMPROVING CHEMICAL COATING  
ON ALUMINUM**

Michael J. Pryor, Spokane, Wash., assignor to Kaiser Aluminum & Chemical Corporation, Oakland, Calif., a corporation of Delaware

No Drawing. Application June 21, 1957  
Serial No. 667,295

5 Claims. (Cl. 148—6.16)

This invention relates generally to the art of coating 15 certain aluminum and aluminum alloy products. More particularly, the invention pertains to an improved process for enhancing the corrosion resistance of chemically coated aluminum and aluminum alloy products of a nature such that entrapment corrosion presents a major 20 problem.

Although the natural oxide film that forms on aluminum and aluminum surfaces affords protection to the metal under ordinary circumstances, severe climatic conditions, such as humid and salt-laden atmospheres, decreases this protection. In order to enhance the corrosion characteristics of aluminum, a number of processes for producing a substantially integral chemical coat upon the aluminum surface by chemical changes in the surface of the metal have been developed. The chromate-phosphate-fluoride type coatings are outstanding examples of chemical coatings for aluminum and aluminum alloys. Chemical coatings produced in solutions containing phosphate ions, chromate ions and fluoride ions as active coating producing ingredients has received wide spread usage for producing chemical coatings affording good corrosion resistance to aluminum surfaces as well as serving as a satisfactory paint base coating. One such process of coating aluminum is commonly known in the trade as the Alodine process. However, it has been found that with the chromate-phosphate-fluoride coatings the corrosion resistance of the metal, particularly to marine atmospheres, is impaired when the product is of such a nature that solid deposits may become easily entrapped. This corrosion is attributed to the presence of non-uniform concentrations of residual hexavalent chromium ions in the chromate-phosphate-fluoride film. These non-uniform hexavalent chromium concentrations may be present either initially or may develop subsequently during service in corrosive atmospheres. The differences in concentration of soluble oxidizing ions in adjacent regions within the coating will lead to the establishment of aggressive local corrosion cells. The weak points in the coating where more effective leaching by the action of rain takes place would contain lower concentrations of oxidizing ions and therefore would be particularly vulnerable to a rapid and highly selective pitting corrosion.

Therefore, it is primary object of this invention to provide an improved chemical coating process for aluminum and aluminum alloy products, of a nature such that entrapment corrosion presents a major problem, wherein the chemical coating affords greater corrosion protection.

It is a further object of this invention to substantially reduce or eliminate the differences in concentrations of soluble oxidizing ions in chromate-phosphate-fluoride chemical coatings.

It is also an object of this invention to provide an improved chemical coating process for aluminum and aluminum alloy products, of a nature such that entrapment corrosion presents a major problem, wherein the concentration variations of soluble hexavalent chromium ions

2

within the coating are reduced or substantially eliminated.

These and other objects and advantages of the invention will be apparent from the ensuing detailed description of the invention.

The invention is based upon the discovery that treatment of chromate-phosphate-fluoride coatings produced on aluminum and aluminum alloy products, wherein soluble hexavalent chromium ions may be present within said coating, with a solution containing reducing ions, that is, a final reducing rinse, will reduce or substantially eliminate the presence of these hexavalent chromium ions. The reducing rinse should contain a powerful reducing agent that does not give insoluble oxidation products and lies within the pH range of about 3.0 to 7.0. An example of a preferred reducing agent is a sodium bisulfite solution containing from about 15 to 150 ounces of sodium bisulfite per 100 gallons of water, however, other reducing agents are contemplated within the scope of the invention. While the above ranges of sodium bisulfite concentration are preferred, concentrations as low as one ounce of sodium bisulfite per 100 gallons of water and as high as 300 ounces of sodium bisulfite per 100 gallons of water may be used to reduce residual hexavalent chromium ions. The aluminum product after being coated with the chromate-phosphate-fluoride coating may be immersed in a tank containing the sodium bisulfite solution, or it may be spray rinsed with the sodium bisulfite solution. In the case of spray rinsing a suitable commercial mixing valve may be used whereby concentrated sodium bisulfite is mixed in the water sprays in the desired concentration. The operating temperature of the sodium bisulfite solution is not critical. After treatment with the sodium bisulfite solution, the coated surfaces are then dried.

In the production of chromate-phosphate-fluoride coatings on aluminum and aluminum alloy products the aluminum surface is treated with an acid aqueous solution containing dichromate ions, phosphate ions, fluoride ions and hydrogen ions. The coating solution may be maintained at any temperature from ordinary room temperature to 180° F. or more, the action of the solution being accelerated by heat. The usual time of treatment to produce the coating ranges from 1 to 2 minutes to 5 to 10 minutes, depending upon the temperature of the solution. Heretofore, it has been the usual practice to rinse the coated surfaces with a dilute chromic acid solution containing from  $\frac{1}{2}$  to 8 ounces of chromic acid per 100 gallons of water, after which the surfaces are dried. As taught by the instant invention, substituting the oxidizing rinse of dilute chromic acid solution with a reducing rinse, e.g. a dilute solution of sodium bisulfite, the presence of oxidizing ions within the coating is reduced or substantially eliminated. The following description of tests comparing the corrosion resistance afforded by chromate-phosphate-fluoride coatings with a chromic acid rinse and with a sodium bisulfite rinse in a corrosive marine environment establishes the efficiency of the sodium bisulfite rinse in reducing corrosion.

60 Samples of a louvered screen of the type known as "Shade Screen," 12 inches square fabricated from 0.008 inch thick 5052 aluminum alloy (containing 2.5% magnesium as a main alloying element) were coated with a chromate-phosphate-fluoride coating in the conventional manner. Half of the samples were rinsed in dilute chromic acid according to conventional practice before drying. The remaining samples were rinsed in a room temperature solution containing 133 ounces of sodium bisulfite in 100 gallons of water. The samples were tested by exposure to a corrosive marine atmosphere at Daytona Beach, Florida. The samples were partly sheltered by an

overhang to accentuate the pickup of wind blown deposits.

After three months the samples rinsed with chromic acid showed perforations of the ribs and louvers, while those samples rinsed in sodium-bisulfite showed no perforations. After nine months exposure, the samples rinsed in chromic acid showed an average of 25 broken ribs and louvers per sample, whereas those rinsed with sodium-bisulfite showed no broken ribs or louvers. These tests under closely simulated service conditions clearly demonstrate the marked superiority of a reducing rinse for products such as louvered aluminum screen.

Although the invention is shown specifically in the above example as applying to the chromate-phosphate-fluoride type of chemical coating, it is not to be construed that the invention is necessarily limited thereto. The invention applies to any chemical coating for aluminum and aluminum alloy products wherein soluble strongly oxidizing ions may be incorporated in the coating in a non-uniform manner and wherein these non-uniform concentrations may be responsible for aggressive local cell corrosion.

Various modifications of processing conditions and in solution compositions permitting the substantial realization of the results herein set forth are deemed within the spirit of the invention and the scope of the appended claims.

What is claimed is:

1. In a process for chemically coating aluminum and aluminum alloy products, of a nature such that entrainment corrosion presents a major problem, wherein said products are subjected to the action of an acid aqueous solution containing chromate ions, phosphate ions and

fluorine ions as active coat-forming constituents to produce a coating on said surfaces, the improvement comprising the step of treating said coating with a rinsing solution containing a reducing agent that does not give insoluble oxidation products, said solution having a pH of about 3.0 to 7.0.

2. In a process for chemically coating aluminum and aluminum alloy products of a nature such that entrainment corrosion presents a major problem, wherein said products are subjected to the action of an acid aqueous solution containing chromate ions, phosphate ions and fluorine ions as active coat-forming constituents to produce a coating on said surface, the improvement comprising the step of treating said coating with a dilute rinsing solution of sodium bisulfite.

3. A process according to claim 2 wherein said sodium bisulfite solution lies within the pH range of from about 3.0 to 7.0.

4. A process according to claim 3 wherein the concentration of sodium bisulfite in said rinsing solution ranges from 1 to 300 ounces of sodium bisulfite per 100 gallons of water.

5. A process according to claim 3 wherein the concentration of sodium bisulfite in said rinsing solution ranges from 15 to 150 ounces of sodium bisulfite per 100 gallons of water.

References Cited in the file of this patent

UNITED STATES PATENTS

|           |                 |               |
|-----------|-----------------|---------------|
| 2,737,498 | Frasch          | Mar. 6, 1956  |
| 2,768,104 | Schuster et al. | Oct. 23, 1956 |
| 2,777,785 | Schuster et al. | Jan. 15, 1957 |